

Sept. 3, 1963

S. M. GRISWOLD

3,102,837

STIFFENER MATERIAL FOR SHOES

Filed March 13, 1961

Fig. 4



Fig. 2



Fig. 1



Fig. 3



Inventor  
Stanley M. Griswold  
By his Attorney

Benjamin C. Pollard

# United States Patent Office

3,102,837

Patented Sept. 3, 1963

1

3,102,837

## STIFFENER MATERIAL FOR SHOES

Stanley M. Griswold, Newton, Mass., assignor, by mesne assignments, to United Shoe Machinery Corporation, Boston, Mass., a corporation of New Jersey

Filed Mar. 13, 1961, Ser. No. 95,423

8 Claims. (Cl. 162—108)

This invention relates to improvements in solvent-activatable sheet stiffener material, particularly material for stiffening end portions of shoes and in a method of making such material.

In my co-pending application for United States Letters Patent, Serial No. 847,550, filed October 20, 1959, there is disclosed a solvent-activatable sheet stiffener material comprising a water-laid layer of intermixed fibers and particles of a stiffening agent soluble at room temperature in an organic solvent. The layer is formed by draining a furnish of fibers containing stiffening agent particles dispersed therein through a thin, relatively open fibrous sheet to which the layer becomes attached by interspersion of fibers. This composite sheet material is effective for its intended purposes and is low in cost.

However, there has been some tendency for displacement of stiffener particles from surface portions of the stiffener material; and although the loss of stiffener particles is not great enough to interfere with the operation of the material, nevertheless, it is undesirable. A further difficulty has been a tendency of the sheet to delamination during handling prior to activation.

In my prior copending application for United States patent, Serial No. 817,191, filed June 1, 1959, now U.S. Patent 3,021,240 of February 13, 1962, there is disclosed a treatment of such a stiffener sheet which in some measure eliminates these difficulties. The treatment there disclosed involves application of a limited amount of solvent to the stiffener sheet in semi-isolated areas on a surface of the sheet material as by spattering or by use of a knurled roll. This treatment produces in the material, beneath the areas of activation, a partial fusion of the stiffening agent particles in an inclusive formation narrowing in cross section depthwise of the material. The effect of this treatment is to render the material firmer and to reduce dusting, i.e. loss of stiffener particles to a considerable extent. However, areas which have not been solvent treated are still prone to lose stiffener particles and the speed of activation of the sheet by solvent and the development of a tacky surface is interfered with to some extent since the prior solvent treatment of the stiffener particles has altered their shape and caused limited agglomeration so that they are no longer as available to attack by solvent as in their original condition. Also, since the incursive formations narrow in cross section depthwise of the material, the firming of the material is irregular and the ability to be skived may not be satisfactory for all purposes.

It is an object of the present invention to provide economical water-laid sheet material comprising fibers and coalescible particles of plastic which is more resistant to loss of particles of stiffening agent without loss of ability to develop surface tack on activation and which possesses improved ability to be skived to a uniform thinly tapering edge.

To this end and in accordance with a feature of the invention, the character of the sheet stiffener is improved and displacement of stiffener particles is substantially eliminated by holding the fibers and particles in associated relation by binder deposited on said fibers and particles but not closing or markedly interfering with the existing porous nature of the sheet stiffener material.

The application of binders to fibrous sheet material

2

presents special problems where it is necessary that the sheet remain porous for later impregnation by a solvent activator. Treatment of surfaces of stiffener sheet material with organic solvent solutions involves the difficulties of using a solvent which will not attack the stiffener particles, and of avoiding the development of an impervious surface coating of binder while at the same time securing the desired deposit in depth of the binder on the fibers and particles. Treatment of stiffener sheet material with an aqueous dispersion of a binder ordinarily results in a deposit of the binder material only in a thin layer near the surface. Here also the desired depth of impregnation has not been obtained.

It is a further object of the present invention to provide a simple and inexpensive method for making a water-laid sheet of fibers and stiffener particles in which the binder will penetrate and effect the desired action on fibers and particles and give the desired character of sheet throughout at least a substantial portion of the thickness of the sheet stiffener material.

To this end and in accordance with a further feature of the invention, an aqueous dispersion of fibers and coalescible particles of a water insoluble plastic is strained through a foraminous surface to form a layer of fibers with particles distributed therethrough, and the web so obtained is treated, while still wet, with an aqueous dispersion of a binder to impregnate the web to a depth of a substantial portion of its thickness. On drying the impregnated web, the binder forms a coherent deposit on the fibers and particles to hold them in associated relation without significantly reducing the porosity of the web. This deposit in depth provides a marked improvement in the ability of the stiffener sheet material to be skived. Also, the binder material in the impregnated portion is in a form and location readily acted on by solvent to create a tacky surface on the stiffener material when the material is activated by solvent.

Other features and advantages of the invention will be understood more fully from the following detailed description taken in connection with accompanying drawings in which:

FIG. 1 is a partial section, greatly enlarged, of a sheet of stiffener material constituting one embodiment of the present invention;

FIG. 2 is an exploded angular view of a portion of a sheet of the type shown in FIG. 1;

FIG. 3 is a diagrammatic elevational view, with parts broken away, of a modified screen cylinder type paper-making machine illustrating the manufacture of a sheet material according to the present invention; and

FIG. 4 is a partial section, greatly enlarged, of a laminate of two composite sheets of intermixed fibers and plastic particles constituting another embodiment of the present invention.

Referring to FIGS. 1 and 2, the sheet material of the present invention comprises a layer 10 of fibers in which is incorporated coalescible particles of a plastic such as an organic solvent soluble stiffening agent, the layer being formed by filtration from a suitable furnish through a sheet 12 of relatively open, fibrous fabric so that fibers of the layer 10 and the sheet 12 are interspersed at the interface 14 (FIG. 2). Binder material is deposited on the fibers and particles in a portion 16 of the layer 10 from the surface of the layer 10 opposite the sheet 12 depthwise into the layer a substantial portion of the entire thickness of the layer, preferably at least one-third of the thickness.

The fiber content of the layer 10 may comprise any suitable papermaking fibers or mixture of fibers such as—cotton, nylon, jute, hemp, hair, wool, kraft or sulfite pulp or asbestos. I have found that kraft paper pulp fibers

have adequate strength and form a very satisfactory product.

The plastic material used in a sheet material intended for shoe stiffening suitably comprises particles of a normally solid, resilient, high molecular weight material soluble at room temperature in a volatile organic solvent and may include, for example, organic solvent soluble resinous polymers and copolymers of ethylenically unsaturated monomers such as, the monovinyl aromatic hydrocarbons of the benzene series including polystyrene and polyvinyl toluene, polyvinyl acetate and the acrylate and methacrylate polymers. Cellulose derivatives, such as cellulose acetate, natural resins, such as modified rosin and the like may also be used alone or in combination. For uses other than shoe stiffening, the foregoing or other coalescible plastics insoluble in the furnish may be used alone or in mixtures depending on the properties desired.

The furnish 18 is an aqueous dispersion and ordinarily the plastic particles will be selected from largely or entirely water-insoluble materials. However, it is also possible to introduce additives to the furnish which reduce the solubility of desirable plastics possessing some solubility in water.

The particles of plastic may be produced by pulverizing scrap plastic material, for example the scrap resulting from the manufacture of polystyrene lenses which is now commonly available. Many plastic materials including polystyrene and polyvinyl toluene may also be employed in the form of small beads made by known suspension polymerization techniques.

It has been found that the presence of the plastic particles materially increases the ease of draining of the furnish over identical furnishes not containing the plastic particles. Also, the size and shape of the plastic particles has an effect both on the ease of the draining of the furnish, on the ability of the dried material to accept solvent and on the softening effect of the solvent.

Thus, polystyrene particles produced by pulverizing scrap polystyrene lens material in a rotary pulverizer have typically a particle size distribution extending from the size of the pulverizer screen openings down to fine powder. Such pulverized material, mixed with water and fiber in a furnish and strained on a screen, usually produces a sheet somewhat more dense, with slower filtration and slower uptake of activating solvent than a sheet made with plastic in the form of fairly uniform beads of equivalent size. These differences are accentuated where the larger particles are screened out of the pulverized material. On the other hand, small pulverized particles or beads in a sheet tend to soften more rapidly upon application of solvent than larger particles or beads because of the greater surface to volume ratio. It has been found that in order to obtain effective draining of liquid from the fiber and particle layer deposited on a screen to enable rapid and economical manufacturing and at the same time to form a sheet which is readily and completely activatable by solvent within the time available in shoe manufacturing processes, it is important that the particle size distribution be as follows: at least 98% passing a No. 40 sieve, 70% to 90% passing a No. 100 sieve, and from 10% to 30% passing a No. 170 sieve, the percentages being by weight of the original mass of particles and the sieves being of the Standard Screen Series, U.S. Bureau of Standards, 1919.

The proportion of plastic particles to fiber may be varied considerably, but for most purposes I find that a ratio of about 1 to 5 parts by weight of plastic particles to one part of fiber is most suitable.

In making a sheet according to one form of the present invention, the plastic particles and fiber are beaten up with a suitable quantity of water to form an aqueous dispersion or furnish. The furnish is strained through a sheet 12 of relatively open fibrous fabric disposed on a support, usually a wire screen 20. However, the function of the screen 20 being merely to support the fibrous

fabric sheet 12, it may conveniently have a larger mesh than usual paper making screens. In fact, the support for the facing sheet may be in any form which provides suitable backing for the sheet 12 while permitting filtration through the fibrous fabric sheet.

The fibrous fabric sheet 12 should be thin, relatively open and flexible yet strong. The open character of the sheet is important in relation to its filtering function in permitting drainage of the water of the furnish while holding back the fiber and plastic particles. This character is also involved in providing adequate attachment of the sheet 12 and the layer 10 of fibers deposited thereon since an open sheet permits, during such filtration, inter-spersion of fibers of the sheet and of the water-laid fibrous layer so that when dry the inter-spersion of the fibers forms a means of attachment between the sheet and the layer deposited thereon. The sheet 12 may be woven or non-woven and may be made from cotton, hemp (e.g. rope paper) or other fibers. If any bonding agent is used in a nonwoven fabric, it should be insoluble in water so that the fibers will not disintegrate. An inexpensive woven fabric such as "tobacco cloth" may be employed. Relatively open non-woven rayon fiber fabric is also useful. This fabric comes in a number of weights and thicknesses ranging from about 8 to 30 grams per square yard and from about 3 to about 8 mils in thickness. I have found suitable fabric which is about 8 grams per square yard in weight and about 3½ mils in thickness.

After sheeting out the furnish to form a layer of desired thickness, water may be removed mechanically from the sheet to reduce the amount which must later be evaporated. Removal of water may be effected by suction and/or by squeezing the sheet between rolls 22. While the composite sheet is still wet, an aqueous dispersion of a binder is applied preferably by a reverse rotating coating roll 24 to the surface of the sheet opposite the surface on which the fabric 12 is secured. It appears that the water content of the web holds the fibers in a more extended relation than would be the case in a dry web and also the water eliminates difficulties caused by dry webs, particularly difficulties of penetration of the binder dispersion into the fiber layer.

The binder may be any liquid solution or dispersion of a material capable of forming a coherent deposit to hold the fibers and particles together. But it is preferred to use a binder which will have certain rubbery characteristics for more effective improvement of the hand of the sheet, i.e. will have the ability to hold the fibers and particles together even where the sheet is subjected to limited flexing. Likewise, it is desirable that the binder be capable of at least partial solution or swelling to a tacky condition when the stiffener is activated by organic solvent. A rubbery copolymer of styrene and butadiene containing from about 30% to 50% of butadiene is a desirable component of the binder and is readily commercially available as a latex, i.e. an aqueous dispersion. It is found that the ability to develop surface tack, the effectiveness of the binder as an aid in improving the character of the stiffener sheet before activation, and in increasing strength and stiffness after activation are improved through the incorporation with the rubbery copolymer latex of a substantial proportion of a latex of a high styrene content butadiene-styrene copolymer, i.e., a copolymer in which the styrene content may be from 50 to 95%. Suitable mixtures of the latices may comprise from about 30% to about 90% by weight solids of the rubbery copolymer with about 10% to 70% by weight solids of the high styrene content copolymer. Latices having a solids content of from about 5% to 15% have been found useful for impregnating a fiber and plastic particle layer according to the present invention. Effective impregnation to achieve the desired results has involved applying from about 0.2 to about 2 oz. of the copolymer solids per sq. ft. of the layer. This impregnation will penetrate at

least  $\frac{1}{3}$  of the thickness of the layer and may extend throughout the thickness of the layer.

After impregnation, the sheet is then dried and may then be rolled to smooth and compact it to about  $\frac{2}{3}$  of its original thickness.

Laminated sheet material constituting another aspect of the present invention (see FIG. 4) includes two or more composite sheets comprising a water-laid layer 10 of intermixed fibers and plastic or resinous particles and an open woven or non-woven reinforcing fabric 12, the fibers of the fibrous layer 10 being interspersed with fibers of the fabric 12 to form a mechanical union holding the layer 10 and the fabric 12 together. A second composite sheet of a water-laid layer 10 of intermixed fiber and plastic or resinous particles and fabric 12 is secured to the first composite sheet by a layer 26 of an adhesive with the fabric layers adjacent. An adhesive will be used which is not unduly softened by solvent to which the laminate may be exposed. Preferably the adhesive is somewhat rubbery to insure that the laminate is flexible and is resistant to delamination when flexed.

Apparatus useful for supporting the fabric sheet 12 for straining a furnish 18 to form a felted fibrous sheet 10, comprises a modified cylinder-type papermaking machine 28 diagrammatically illustrated in FIG. 3. As there shown, the machine 28 comprises a vat 30 with a flow box 32 at one end for insuring a smooth supply of furnish to the interior of the vat 30. The flow box 32 is of conventional type comprising a bottom wall 34 and an end wall 36 of which the upper edge 38 is adjustable heightwise to regulate flow of furnish from the interior of the flow box 32 to the interior of the vat 30. The bottom wall 34 and end wall 36 extend across the interior of the vat 30 and cooperate with the side walls 40 and end wall 42 of the vat 30 to define a chamber 44 into which furnish is fed through the pipe 46. A cylinder 48 is rotatably mounted in the vat 30 and is provided with means for driving it (not shown). A pipe 50 for withdrawing liquid is disposed in the interior of the cylinder 48. The cylinder 48 differs from conventional papermaking cylinders in that the wire screen 20 on its surface is of substantially larger mesh. It is desirable that the openings in the screen be at least about  $\frac{1}{6}$  greater than the dimension of the largest plastic or resin particles of the furnish to prevent plugging of the screen by the particles. It should be noted that the screen openings may in some instances be somewhat reduced by reinforcing wires and the screen opening size referred to is the actual screen opening. Depending on the size of the plastic particles, there may be used screens from size No. 12 to size No. 30 (U.S. Bureau of Standards, Standard Screen Series, 1919).

For the first operation to form a mechanically linked fabric and felted fiber-plastic particle sheet, fabric 12 is withdrawn from a roll 52, passed around a roller 54 which lays it down on the screen 20 of the cylinder 48 and the fabric 12 is carried around the cylinder 48 by rotation of the cylinder. As shown in FIG. 3, the water component of the furnish passes through the fabric 12 to the interior of the cylinder 48 leaving behind a layer 10 of intermixed fibers and plastic particles. Fibers from the furnish 18 deposited on the fabric 12 penetrate and become entangled with the fibers of the fabric 12 to attach mechanically the deposited intermixture of fibers and plastic particles to the fabric 12. When the fabric 12 and the attached felted layer 10 of fibers and plastic particles have passed nearly around the cylinder 48, they are lifted from the surface of the cylinder by a couch roll 56 and felt 58 and carried up with the felt over the rollers 60 and 62. From the roller 62, the composite of the fabric 12 and felted layer 10 is passed between squeeze rolls 22 which mechanically express a portion of the water content and then passes over a coating roll 24 of which the lower portion dips into a body 64 of binder liquid in the tray 66. The roll 24 rotates in a direction so that its surface is mov-

ing counter to the direction of movement of the composite sheet so that substantially the entire quantity of binder liquid picked up by the surface of the roll 24 is transferred and serves to impregnate the fiber layer 10.

5 After the step of impregnation, the sheet is dried by suitable drying means such as heated drying rollers 68.

Where a laminated stiffener is to be manufactured, the surface of the fabric 12 of a composite sheet is coated with a high viscosity adhesive layer 26. Useful adhesives include natural or synthetic rubber latices. After application of the layer 26 of this adhesive, to the fabric 12, the fabric covered surface of a second composite sheet is pressed against the adhesive layer 26 and the adhesive allowed to dry to form a firm bond between the two sheets.

10 15 The following example is given to aid in understanding the invention, but it is to be understood that the invention is not restricted to the particular materials, purposes or procedures set forth in the example.

Example.—A furnish was prepared by beating kraft pulp in water using a Hollander type beater device. The furnish was adjusted to a fiber content of 0.14% fiber and there was then introduced polystyrene beads of which 100% pass through a No. 16 screen (screen opening 0.047"), 99.7% pass through a No. 40 screen (screen opening 0.0165"), 90% pass through a No. 100 screen (screen opening 0.006"), and 15% pass through a No. 170 screen (screen opening .0035") in amount to bring the resin content of the furnish to 0.35%.

20 25 30 Tobacco cloth was drawn from a roll and laid down on the screen of a cylinder type papermaking machine by a roll resting on the screen at the top of the cylinder. The screen was No. 14 (screen opening 0.0555"). The cloth was brought around the cylinder and around a couch roll and felt at the top of the cylinder.

35 40 45 The cylinder which was 18" in diameter was set in rotation at about 3 r.p.m. and furnish introduced into the flow box of the machine to fill the vat of the machine nearly to within 2" of the top of the cylinder. The white water from the furnish strained through the cloth on the cylinder screen leaving behind a layer of intermixed fiber and resin. The liquid entering the interior of the cylinder was withdrawn. The layer of intermixed fiber and resin particles increased in thickness as it passed around the cylinder and was lifted off the screen as a composite sheet 50 by the couch roll and felt. The composite sheet was passed between rolls to squeeze water from it. In the sheet, the fibers of the intermixed fiber and resin particle layer were interspersed with the fibers of the tobacco cloth to an extent sufficient to hold the fiber and resin particle layer firmly to the tobacco cloth.

55 60 65 70 75 78 7.8 gallons of a 40% solids latex of a copolymer of equal parts by weight of butadiene and styrene and 7.8 gallons of a 45% solids latex of a copolymer 80% styrene and 20% butadiene were mixed with 3.9 gallons of a 10% solution of Aquarex-D and 80.5 gallons of water. The mixture was supplied to the tray into which the coating roll dipped. The composite sheet of intermixed fiber and resin particle layer and tobacco cloth was passed over the coating roll with the fiber and resin particle layer against the roll. The roll rotated in a direction so that its surface moved counter to the direction of movement of the composite sheet and the surface of the roll picked up the mixed latex composition from the tray and deposited it on the surface of the layer. It was observed that the deposited latex penetrated into the surface of the layer promptly after application. The speed of the roller was controlled to provide a deposit of about .6 oz. of solids of the latex per square foot of the composite sheet. After the step of impregnation, the sheet was dried by passing it around the heated drying rollers.

The dry composite sheet was coated on the cloth side with a thickened natural rubber latex (60% solids) an excess of the latex being applied and scraped off with a doctor blade. Thereafter a second composite sheet was

assembled with its fabric surface against the deposit of rubber latex on the first composite sheet.

After the latex adhesive had set, a box toe blank was cut from the laminate. The edges of the box toe blank were skived in a standard skiving machine and it was found that a thin uniform firm edge was obtained. The surfaces of the blank did not tend to lose the particles of the resin and the sheet itself was capable of the flexing normally encountered in shoe making procedures without delamination. The box toe blank was treated with a solution comprising 8 parts of methyl ethyl ketone and 16 parts of toluol. The solution rapidly and completely penetrated and softened the laminate and brought the surfaces of the laminate to a tacky condition. The activated blank was placed in the toe of the shoe, the shoe was lasted and the stiffener allowed to harden. The toe of the shoe was found to be stiff and resilient and to maintain its shape under the conditions encountered in use.

Having thus described my invention, what I claim as new and desire to secure by Letters Patent of the United States is:

1. In a hardenable sheet material for stiffening end portions of shoes comprising a porous layer of water-laid fibers intermixed with discrete particles of normally solid, organic solvent-soluble coalescible stiffening agent with said particles being present in the ratio of from about 1 to about 5 parts by weight to 1 part by weight of fibers, the improvement including a coherent deposit of a binder on said fibers and particles from one surface in to a depth of a substantial portion of the thickness of said layer and holding said fibers and particles in associated relation but not closing the pores of said layer, said binder being swellable to tacky condition by an organic solvent activator for said sheet material.

2. In a hardenable sheet material for stiffening end portions of shoes comprising a porous layer of water-laid fibers intermixed with discrete particles of normally solid, organic solvent-soluble coalescible stiffening agent with said particles being present in the ratio of from about 1 to about 5 parts by weight to 1 part by weight of fibers, the improvement including a coherent deposit of a binder on said fibers and particles from one surface in to a depth of a substantial portion of the thickness of said layer and holding said fibers and particles in associated relation but not closing the pores of said layer, said binder comprising a rubbery copolymer of styrene and butadiene reduceable to tacky condition by an organic solvent activator for said sheet material.

3. In a hardenable sheet material for stiffening end portions of shoes comprising a porous layer of water-laid cellulosic paper-making fibers intermixed with coalescible discrete particles of normally solid, organic solvent-soluble thermoplastic polymer resin with said particles being present in the ratio of from about 1 to about 5 parts by weight to 1 part by weight of fibers and a relatively open fibrous fabric on a face of said layer with fibers of said layer and fibers of said fabric interspersed at the interface between them to provide a mechanical link holding said layer to said fabric, the improvement including a coherent deposit of a binder on said fibers and particles from the other face of said layer in to a depth of  $\frac{1}{3}$  of the thickness of said layer and holding said fibers and particles in associated relation but not closing the pores of said layer, said binder comprising a rubbery copolymer of styrene and butadiene reduceable to tacky condition by an organic solvent activator for said sheet material.

4. In a hardenable sheet material for stiffening end portions of shoes comprising a porous layer of water-laid cellulosic paper-making fibers intermixed with coalescible discrete particles of normally solid, organic solvent-soluble thermoplastic polymer resin with said particles being present in the ratio of from about 1 to about 5 parts by weight to 1 part by weight of fibers and a rela-

tively open fibrous fabric on a face of said layer with fibers of said layer and fibers of said fabric interspersed at the interface between them to provide a mechanical link holding said layer to said fabric, the improvement including a coherent deposit of a binder on said fibers and particles from the other face of said layer in to a depth of  $\frac{1}{3}$  of the thickness of said layer and holding said fibers and particles in associated relation but not closing the pores of said layer, said binder comprising from about 30% to about 90% by weight of a rubbery copolymer of styrene and butadiene and from about 10% to about 70% by weight of a copolymer of butadiene and styrene in which the styrene content is from 50% to 75% reduceable to tacky condition by an organic solvent activator for said sheet material, said binder being present to the extent of from about 0.2 to about 2 ounces per square foot of the surface of said layer.

5. In a hardenable sheet material for stiffening end portions of shoes comprising a porous layer of water-laid cellulosic paper-making fibers intermixed with coalescible discrete particles of normally solid polystyrene resin with said particles being present in the ratio of from about 1 to about 5 parts by weight to 1 part by weight of fibers and a relatively open fibrous fabric on a face of said layer with fibers of said layer and fibers of said fabric interspersed at the interface between them to provide a mechanical link holding said layer to said fabric, the improvement including a coherent deposit of a binder on said fibers and particles from the other face of said layer in to a depth of  $\frac{1}{3}$  of the thickness of said layer and holding said fibers and particles in associated relation, but not closing the pores of said layer, said binder comprising from about 30% to about 90% by weight of a rubbery copolymer of styrene and butadiene and from about 10% to about 70% by weight of a copolymer of butadiene and styrene in which the styrene content is from 50% to 75% reduceable to tacky condition by an organic solvent activator for said sheet material, said binder being present to the extent of from about 0.2 to about 2 ounces per square foot of the surface of said layer.

6. In a hardenable sheet material for stiffening end portions of shoes comprising a laminate of two composites of porous layer and open fibrous fabric, said composites being held in laminated relationship with the fibrous fabric covered surfaces adjacent to each other by a rubber base adhesive, said porous layers comprising water-laid cellulosic papermaking fibers intermixed with coalescible discrete particles of normally solid polystyrene resin with said particles being present in the ratio of from about 1 to about 5 parts by weight to 1 part by weight of fibers and a relatively open fibrous fabric on a face of said layer with fibers of said layer and fibers of said fabric interspersed at the interface between them to provide a mechanical link holding said layer to said fabric, the improvement including coherent deposits of a binder on said fibers and particles from the other faces of said layers in to a depth of  $\frac{1}{3}$  of the thickness of said layers and holding said fibers and particles in associated relation, but not closing the pores of said layers, said binder comprising from about 30% to about 90% by weight of a rubbery copolymer of styrene and butadiene and from about 10% to about 70% by weight of a copolymer of butadiene and styrene in which the styrene content is from 50% to 75% reduceable to tacky condition by an organic solvent activator for said sheet material, said binder being present to the extent of from about 0.2 to about 2 ounces per square foot of the surface of said layers.

7. In a method of making hardenable sheet material for stiffening end portions of shoes comprising the steps of forming an aqueous dispersion of fibers and discrete particles of a normally solid thermoplastic water insoluble organic solvent-soluble coalescible stiffening agent, said particles being present in the ratio of from about one to

about five parts by weight to one part by weight of fibers, straining the dispersion through a thin relatively open fibrous fabric on a foraminous surface to deposit on said fabric a layer of fibers with said particles distributed therethrough and with fibers of said layer interspersed with fibers of said fabric to provide a mechanical link holding said layer to said fabric, removing water from the layer, consolidating said layer, removing the composite of fabric, fiber and particles from said foraminous surface as a wet web, the improvement including applying an aqueous dispersion of a binder to the surface of said wet web opposite said fabric to impregnate said web to a depth of at least about one-third of the thickness of said layer and drying said web to form a coherent deposit of said binder on said fibers and particles to hold them in associated relation but not closing the pores of said layer, said binder being swellable to tacky condition by an organic solvent activator for said sheet material.

8. In a method of making hardenable sheet material for stiffening end portions of shoes comprising the steps of forming an aqueous dispersion of fibers and coalescible particles of a normally solid, thermoplastic water-insoluble, organic solvent-soluble resinous polymer of a monovinyl aromatic hydrocarbon of the benzene series, said particles being present in the ratio of from about one to about five parts by weight to one part by weight of fibers, and said particles being of a size distribution as determined with U.S. Standard Sieves in which at least 98% will pass through a No. 40 sieve, from about 70% to about 90% will pass through a No. 100 sieve and from about 10%

5 to about 30% will pass through a No. 170 sieve, straining the dispersion through a thin relatively open fibrous fabric on a foraminous surface to deposit on the fabric a layer of fibers with said particles distributed therethrough and with fibers of said layer interspersed with fibers of said fabric to provide a mechanical link holding said layer to said fabric, removing water from the layer, consolidating said layer, removing the composite of fabric, fiber and particles from said foraminous surface as a wet web, the improvement including applying a latex of a rubbery copolymer of styrene and butadiene to the surface of said wet web opposite said fabric to impregnate said web to a depth of at least one-third of the thickness of said layer and drying said web to form a coherent deposit of said styrene-butadiene copolymer on said fibers and particles to hold them in associated relation but not closing the pores of said layer, said polymer being swellable to tacky condition by an organic solvent activator for said sheet material.

10

## References Cited in the file of this patent

## UNITED STATES PATENTS

|              |              |                |
|--------------|--------------|----------------|
| 1,731,754    | Richards     | Oct. 15, 1929  |
| 1,861,044    | Ballard      | May 31, 1932   |
| 25 1,921,504 | Chase et al. | Aug. 8, 1933   |
| 1,926,028    | Boughton     | Sept. 12, 1933 |
| 1,945,173    | Woodruff     | Jan. 30, 1934  |
| 1,961,916    | Sherman      | June 5, 1934   |
| 30 1,968,437 | Boughton     | July 31, 1934  |
| 2,076,636    | Hanley       | Apr. 13, 1937  |